

(No Model.)

J. F. MARTIN.

INSULATOR FOR ELECTRIC WIRES.

No. 286,946.

Patented Oct. 16, 1883.

Fig. 1.



Fig. 2.



Fig. 3.



Fig. 4.

Witnesses.

Will R. Oshundro

Frank J. Blanchard.

Inventor.

John F. Martin

By Jno. G. Elliott  
Atty.

# UNITED STATES PATENT OFFICE.

JOHN F. MARTIN, OF CHICAGO, ILLINOIS.

## INSULATOR FOR ELECTRIC WIRES.

SPECIFICATION forming part of Letters Patent No. 286,946, dated October 16, 1883.

Application filed March 12, 1883. (No model.)

*To all whom it may concern:*

Be it known that I, JOHN F. MARTIN, a citizen of the United States, residing in Chicago, county of Cook, and State of Illinois, have invented certain new and useful Improvements in Insulators for Electric Wires, of which the following is a specification.

This invention relates to improvements in electric-wire insulators composed of sheet-paper or woven material rolled to form tubes which are coupled together, so as to provide for each wire of an underground system a separate and continuous chamber.

The object of my invention is to render the tubes compact, strong, and durable, to unite the coils or layers of paper firmly together, and to utilize the means employed for securing said layers together as a means for incorporating in the material a large quantity of some insulating compound which shall tend to render the tube water-proof. To such end, I place together a perforated and an imperforate sheet of paper or other suitable material, and after filling the perforations with some insulating-cement I roll the sheets thus united into tubular form.

In the annexed drawings, Figure 1 represents two sheets combined and partially rolled into tubular form. Fig. 2 shows a section 30 taken through two sheets, with the perforations in one of them filled with cement. Fig. 3 represents one of the sheets having circular perforations. Fig. 4 is a section taken through Fig. 3.

Referring by letter to the several figures of the drawings, in which like letters indicate like parts, A and B denote two sheets of paper, which are placed together, so that they can be manipulated as one sheet. One of these sheets is provided with slots or perforations C, which can be made of any desired shape—as, for example, oblong, as shown in Fig. 1, or circular, as in Fig. 3. The perforations are preferably arranged in parallel rows, with those of one row opposite the spaces between the perforations of the next succeeding row; but it will be evident that they could be otherwise arranged. The sheets can be made of equal thickness, or one can be made

somewhat thicker than the other, as in Fig. 2, 50 in which the perforated sheet A is the thicker of the two. After the sheets have been laid together, as herein shown, the perforations C are filled with some insulating compound or cement and the sheets then rolled to form a 55 tube. The cement filling holds the sheets together, and also holds them in the shape into which they have been rolled. In this way a comparatively large quantity of cement is distributed throughout the material without increasing the thickness of the same, which latter would be the case if the cement were laid on in a layer upon one of the sheets. The tubes thus made can be coupled together, so as to form continuous lines of tubing, the couplings being preferably composed of sleeves, 60 which are fitted upon the ends of the tube-sections.

In other applications which I have made for Letters Patent the tube is shown made of but 70 one sheet, and in one of said applications the sheet is perforated, and the perforations filled with cement before the sheet is rolled into tubular form. Such construction of tube, however, lacks the features of an imperforate 75 sheet constituting the backing for the perforated sheet as herein shown.

Both sheets can be made of paper or some suitable woven material, or one sheet can be made of paper and the other of woven material, as preferred.

The cement employed will preferably consist of asphaltum or asphaltum combined with some suitable material, such as is generally used with asphaltum for the purpose of rendering it hard and durable after it dries.

Having thus described my invention, what I claim, and desire to secure by Letters Patent, is—

An insulator for electric wires, composed of 90 a perforated and an imperforate sheet rolled into tubular form, with the openings of the perforated sheet filled with some insulating compound, substantially as described.

JOHN F. MARTIN.

Witnesses:

W. W. ELLIOTT,  
JNO. G. ELLIOTT.